

## UNITED STATES PATENT OFFICE.

ALBERT L. STILLMAN, OF PLAINFIELD, NEW JERSEY, ASSIGNOR TO THE GENERAL FUEL BRIQUETTE CORPORATION, OF NEW YORK, N. Y., A CORPORATION OF NEW YORK.

## PROCESS OF MANUFACTURING FUEL BRIQUETTES.

No Drawing.

Application filed January 21, 1927. Serial No. 162,681.

This invention relates to the manufacture of briquettes and particularly to fuel briquettes. The principal object of the invention is to provide a new and improved process of manufacturing fuel briquettes by means of which briquettes of high caloric value and of great strength and durability may be produced.

The present invention rests on the discovery that certain types of coal when mixed with a binder consisting of asphalt or pitches which are solid at ordinary temperatures but liquefy at between 110° to 212° F., and the melted liquid with the hot coal are subjected to a severe grinding action, a certain amount of the volatile constituent of the coal is dissolved in the melted binder, and that such solution hastens the subsequent set of the briquette and increases the tendency of the briquette to resist abrasion and breakage.

It is necessary in order to take advantage of this discovery to use coal of a certain type, such as will under conditions of severe grinding and the applied heat, give off some volatile material. Coals of this character are, generally speaking, any of the coals known as soft coals, of which the Pocahontas and New River varieties are particular examples. It is also necessary for the carrying out of the new process that the mixing and grinding action be of considerable intensity such as results for example from the use of a masticator of the type known in Canadian Patent No. 184,646, of May 28, 1918. Such masticators exercise a kneading effect of considerable severity and consequently facilitate that function of the process which is concerned with the extraction of the volatiles from the hot coal during the mixing operation. In order to carry out the process advantageously, it is necessary that the coal under treatment be itself heated to a temperature of the order of 125° F. during its mastication, the temperature of the coal to be high enough to maintain the liquidity of the binding ingredients during the operation. It is therefore of advantage to give the masticator during the operation as much heat insulation as possible and it is of still further benefit if the operation be carried on in the presence of water vapor. One salient prac-

tical effect of the process is to decrease markedly the amount of binder required, 55 inasmuch as dissolved coal substance becomes binder substance.

In a particular example of the process the soft coal, preferably in a comminuted condition, is mixed with asphalt or pitches 60 such as are solid at ordinary temperatures but which liquefy at between 100 and 212° F., the asphalt or pitch serving as the primary binder. The binder material is heated to liquefy it and is then mixed with 65 the coal in about the proportion of 10% binder to 90% coal. The mixture is subjected to a severe or intense grinding action in a masticator which is insulated against substantial heat losses, or is otherwise main- 70 tained in a heated condition during the grinding operation. By maintaining the mixture at a temperature not lower than 125° F. during the grinding thereof and in any event at least high enough to maintain 75 the binder in a liquid state, a certain amount of the volatile constituents of the coal is liberated and is dissolved in the melted binder forming secondary binder substances. After being thus treated, the ma- 80 terial is briquetted.

It is of considerable importance during the grinding operation, to prevent the temperature of the mixture from falling below a degree at which there would be no volatilization of the constituents of the coal, and therefore it is of advantage to give the grinding operation as much heat insulation as possible. The provision of such insulation is preferred because while a similar 90 result could obviously be obtained by the external application of heat to the grinder, such external application would necessarily involve added manufacturing costs.

The efficiency of the process may be still 95 further increased if the grinding operation is performed in the presence of water vapor. Such vapor may be introduced into the masticator through a pipe in the form of steam thus assisting in maintaining the de- 100 sired temperature during the grinding operation.

Having thus described my invention, what I claim and desire to secure by Letters Patent of the United States is:

1. In the process of making fuel bri-

quettes, the improvement which consists in mixing bituminous coal with a bituminous binder heated to a molten condition, and subjecting the mixture at a temperature above 125° F. and in the presence of steam 15 to an intense grinding operation until volatile constituents of the coal are liberated and passed into solution in the molten binder.

5 above the fusion point of the binder and in the presence of water vapor to an intense grinding operation until volatile constituents of the coal are liberated and passed in-  
to solution in the molten binder.

10 2. In the process of making fuel bri-  
quettes, the improvement which consists in

In testimony whereof I have hereunto 20  
set my hand.

ALBERT L. STILLMAN.